

[54] COLOR CATHODE RAY TUBE SCREEN  
STRUCTURE PROVIDING IMPROVED  
CONTRAST

[75] Inventors: Mahlon B. Fisher, Skaneateles;  
Anthony V. Gallaro, Auburn; George  
N. Williams, Seneca Falls, all of N.Y.

[73] Assignee: GTE Sylvania Incorporated,  
Stamford, Conn.

[21] Appl. No.: 412,143

[22] Filed: Nov. 2, 1973

[51] Int. Cl.<sup>2</sup> ..... H01J 29/26; H01J 31/20

[52] U.S. Cl. ..... 313/470; 313/472;  
313/474

[58] Field of Search ..... 313/470, 472, 474

[56] References Cited

U.S. PATENT DOCUMENTS

3,695,871 10/1972 Lange ..... 313/472  
3,748,515 7/1973 Kaplan ..... 313/472

Primary Examiner—John K. Corbin

Assistant Examiner—Rolf Hille

Attorney, Agent, or Firm—Thomas H. Buffton

[57] ABSTRACT

A color cathode ray tube screen structure, having means for enhancing the absorption of ambient light and providing improvement in the contrast of the image display, is comprised of three superimposed substantially continuous window-defining layers of optical filter materials. The primary, secondary and tertiary filter layers have discretely disposed window areas formed therein to expose a pattern of filter areas representing the respective filter materials. The filter windows are of a shaping similar to that of the apertures in a spatially related pattern mask member. Each window exhibits a uniform periphery free of indentations, being so defined by a uniform opaque interstitial encompassment homogeneously made up of the three distinct layers of filter materials. Disposed over the filter windows is a patterned screen of cathodoluminescent phosphor elements, which upon electron excitation produces color-emissions that are colormetrically related to the respective filter windows therebeneath.

7 Claims, 11 Drawing Figures





Fig. 1a



Fig. 1b



Fig. 1c



Fig. 1d



Fig. 1e



Fig. 1f



Fig. 1g



Fig. 2



Fig. 3



Fig. 4



Fig. 5

**COLOR CATHODE RAY TUBE SCREEN  
STRUCTURE PROVIDING IMPROVED  
CONTRAST**

**CROSS REFERENCES TO RELATED  
APPLICATIONS**

This application contains matter disclosed but not claimed in three related United States Patent Applications filed concurrently herewith and assigned to the assignee of the present invention. These related applications are Ser. No. 412,142, now U.S. Pat. No. 3,884,694; Ser. No. 412,145, now U.S. Pat. No. 381,440; and Ser. No. 412,144, now U.S. Pat. No. 3,884,695; all of which were filed in the U.S. Patent Office on Nov. 2, 1973.

**BACKGROUND OF THE INVENTION**

This invention relates to color cathode ray tubes and more particularly to a tube screen structure providing improved contrast of the color image display.

Cathode ray tubes of the type employed in color television applications for presenting multi-color display imagery, usually utilize patterned screens that are comprised of repetitive groups of related phosphor materials. Such groupings are normally disposed as bars, stripes or dots depending upon the type of color tube structure under consideration. For example, in the well known shadow mask tube construction, the screen pattern is conventionally composed of a vast multitude of repetitive tri-color emissive areas formed of selected cathodoluminescent phosphors, which, upon predetermined excitation, produce additive primary hues to provide the desired color imagery. Associated with the screen and spaced therefrom is a foraminous structure or patterned mask member having a vast multitude of discretely formed apertures therein. Each of the apertures in the mask member is related to a specific tri-component grouping of related phosphor areas of the screened pattern in a spaced manner therefrom to enable the selected electron beams traversing the apertures to impinge the proper screen areas therebeneath.

Several approaches have been proposed to increase the contrast ratio of the color screen display. On such proposal to improve contrast by absorbing ambient light is the use of a neutral density filter member in the form of a tinted cover plate which is superposed on the viewing panel of the tube. Since neutral density filters are not appreciably selective in the visible band of the color spectrum, the intended absorptive efficiency can not be fully realized in eliminating the reflective ambient light falling within the spectrum bandpass of the display emission. Another proposal for increasing contrast ratio of the color image display is the utilization of a tinted faceplate or viewing panel per se. Tinting of the faceplate attenuates the light transmission of that member, thereby reducing the evidenced brightness of the phosphor emissions, in addition to absorptive shortcomings similar to those of the aforementioned neutral density filter.

Another approach to improving contrast of the color screen image, particularly in a dot-type patterned screen, has been the development of a screen structure wherein the dot-defining interstitial spacing between the respective color-emitting dots of the screen pattern is formed of an opaque light absorbing material. In essence, each phosphor dot is enclosed or defined by a substantially dark encompassment which collectively comprise a foraminous pattern in the form of a win-

dowed webbing having an array of substantially opaque connected interstices. While this black surround feature reduces the reflected ambient light in the non-fluorescing areas of the screen, it does not reduce the ambient light reflected from the panel areas associated with the phosphor dots, which areas evidence a high degree of reflectivity.

A further proposal for enhancing contrast of the screen display has been the use of optical filter elements disposed relative to the respective color-emitting phosphors comprising the screen pattern. On such optical filter proposal utilizes circular filter elements having large oversize diameters dimensioned so that their outer peripheral portions overlap in a non-uniform manner to produce an irregularly shaped or indented filter area surrounded by a non-uniform interstitial webbing. These variations in the dot surround-webbing effect a variable absorbency of the ambient light thereby detracting from the complete achievement of the intended contrast enhancement.

**OBJECTS AND SUMMARY OF THE  
INVENTION**

It is an object of the invention to reduce the aforementioned disadvantages and to provide an improved screen structure for a color cathode ray tube evidencing improved display contrast.

It is another object to provide an improved color cathode ray tube screen structure having optical filter elements therein surrounded by an opaque interstitial webbing of uniform thickness.

It is another object to provide an improved color cathode ray tube screen structure incorporating optical filter windows therein, each window in the screen structure having a uniform peripheral encompassment free of indentations.

These and other objects and advantages are achieved in one aspect of the invention by a discretely patterned multi-window color screen structure disposed on the inner surface of a cathode ray tube viewing panel. Each of the window areas is surrounded by a uniform opaque interstitial encompassment that exhibits a peripherally defined smoothness free of indentations, such shaping being similar to the shape of the apertures in a spatially related pattern mask member. The screen structure is comprised of a transparent primary layer of a first heat formable optical filter material that is adhered to the inner surface of the viewing panel. This primary layer has open second and third pattern window areas formed therein. A secondary layer of a second heat formable optical filter material is superimposed on the primary layer and the second of the window pattern areas formed therein to provide an array of window-defined second filter elements in the screen structure. The secondary layer has open first and third patterned window areas formed therein whereof the open first window pattern array defines portions of the primary layer to provide a delineation of first filter elements in the screen structure that are free of peripheral indentations. The open third window pattern in the secondary filter layer is superimposed over the open third window pattern in the primary filter layer. A tertiary layer of a third heat formable optical filter material is disposed in a superposed manner over the secondary layer and the open third superposed window pattern areas to provide an array of third filter elements in the screen structure. This tertiary layer has open first and second window patterns superimposed on like window areas in the sec-

ondary layer. The three superimposed optical filter material layers are combined uniformly to provide a substantially opaque uniform interstitial webbing fully surrounding each of the respective filter windows in the color screen structure; each of the windows having a uniform peripheral encompassment free of indentations. This opaquely defined filter windowed structure has three patterns of related cathodoluminescent phosphor elements disposed thereover to complete the color screen structure.

#### BRIEF DESCRIPTION OF THE DRAWINGS

FIGS. 1a and 1b are cross-sectional views illustrating deposition of the primary layer of the first optical filter material;

FIGS. 1c and 1d are cross-sectional views relating to the deposition of the secondary layer of a second optical filter material;

FIGS. 1e and 1f are sectional views illustrating the deposition of tertiary layer of the third optical filter material;

FIG. 1g is a sectional view showing the completed screen structure;

FIG. 2 is a plan view of a partially constructed screen structure taken along the line 2-2 of FIG. 1b showing the primary layer of the first optical filter material and the open second and third patterned window areas formed therein;

FIG. 3 is a plan view of a partially constructed screen structure taken along the line 3-3 of FIG. 1d illustrating the superposed primary and secondary filter material layers and the window elements associated respectively therewith;

FIG. 4 is a plan view of the screen structure taken along the line 4-4 of FIG. 1f showing the relationship of the superposed primary, secondary and tertiary layers of the optical filter materials and the respective filter windows formed therein; and

FIG. 5 is a plan view of the completed screen structure taken along the line 5-5 of FIG. 1g.

#### DESCRIPTION OF THE PREFERRED EMBODIMENT

For a better understanding of the present invention, together with other and further objects, advantages and capabilities thereof, reference is made to the following specification and appended claims in connection with the aforescribed drawings.

The improved discretely pattern multi-window color cathode ray tube structure described herein will be delineated as having substantially round filter window areas therein surrounded by a substantially uniform opaque interstitial encompassment; each of the window areas having a defined peripheral smoothness free of indentations. Other window configurations, such as elongated and ovate shapings, are intended to be in keeping with this disclosure, such configurations being similar to the shape of the apertures in a spatially related pattern mask member. The screen structure so described may be utilized in either post deflection or shadow mask types of color cathode ray tube constructions.

In this instance, a multi-element filter window screen structure 11 of the invention as illustrated in FIGS. 1g and 5 is of the type, for example, as that used in a conventional shadow mask type of color cathode ray tube. As is well known, conventional tubes of this type utilize several electron beams which are directed to converge

at a multi-apertured shadow mask, not shown, and thence pass through the apertures therein to discretely impinge selected areas of the composite screen structure spaced therebeneath. The multi-layered screen structure 11 as shown in FIGS. 1g and 5, is disposed on the inner surface of the cathode ray tube viewing panel 13. The visible light transmissivity of this glass panel is relatively high being preferably in the neighborhood of 90 percent, the light attenuation of the glass per se being inherent to the elemental composition thereof. Attached to the inner surface of this panel is a substantially continuous and substantially transparent primary layer 21 of a first heat formable optical filter material representative of a primary hue. This primary layer has substantially round second and third patterns of related open window areas, 25 and 27 respectively, formed therein each being free of peripheral indentations. The hue of this primary layer is a primary color as, for example, green "g," and is of a first organometallic luster composition as will be more fully explained subsequently in this specification. Superposed on this primary filter layer 21 is a substantially continuous and substantially transparent secondary layer 31 of a second heat formable optical filter material differing in hue from that of the primary layer, as for example, a blue "b" coloration resultant of another or second organometallic luster composition. This secondary layer 31 overlays and fills in the second of the window pattern areas 25 formed in the primary layer 21 to provide an array of window defined second filter elements 26 in the screen structure. Additionally, the secondary layer has first and third patterns of discrete window areas, 33 and 37 respectively, formed therein whereof the first window pattern array 33 defines areal portions of the first or primary layer 21 to provide first filter elements 24 in the screen structure. The third window pattern 37 in the secondary layer 31 is superimposed over the third window pattern 27 in the primary layer 21. A substantially continuous and substantially transparent tertiary layer 41 of a third heat formable optical filter material is superposed over the secondary layer 31 and fills in the third window pattern areas 37 therein and the underlying window pattern areas 27 to provide the array of defined third filter elements 36 in the screen structure 11. This tertiary layer 41 is of a hue differing from that of the primary and secondary layers, as for example red "r," and is formed of a third organometallic luster material having open first and second window patterns, 43 and 45 respectively, that are superposed on like window areas 33 and 25, in the secondary and primary filter layers 31 and 21 respectively. The three superimposed layers 21, 31 and 41 of diverse primary color optical filter materials comprising the multi-window structure 11 are combined in a discrete manner to provide a substantially opaque uniform interstitial webbing 49 that fully surrounds each of the respective filter windows in the screen structure by an opaque uniform peripheral encompassment that is free of indentations. Disposed over these respective filter window areas of the screen structure are patterned groupings of compatible green "G," blue "B" and red "R" cathodoluminescent phosphor elements, which upon electron excitation produce color-emissions that are colorimetrically related to the respective filter windows 24 "g," 26 "b," and 36 "r" therebeneath. The color emissions of the phosphor materials are selectively enhanced by transmission through the associated filtering components.

Portions of the process for fabricating the aforescribed interstitially defined first 24, second 26 and third 36 filter window areas comprising the color cathode ray tube screen structure 11 are delineated in FIGS. 1a through FIG. 1f of the drawings.

Prior to the initiation of the screen structure fabricating process, the viewing or face panel portion 13 of the cathode ray tube is cleaned in a normal manner by washing particularly the interior of the panel with a 5 to 10 percent aqueous solution of hydrofluoric acid, whereupon the panel is water rinsed and dried. The first step in fabrication of the screen structure entails uniformly coating the interior surface of the panel 13 with a primary layer of a liquid mixture 19 of a positive photosensitive resist material and a first organometallic luster compound. Positive photosensitive resist is a light activated material that, when exposed to actinic radiation, such as uv, becomes polymerically degraded thereby acquiring solubility in its development solvent. A typical positive photosensitive resist material is one such as that designated AZ-111, distributed by Shipley Company, Incorporated, Newton, Mass. The first organometallic luster compound, as mixed with the positive photosensitive resist, is selected from the group of compounds known as liquid luster preparations. Such compositions are base metal organic solutions of metals such as tin, iron, bismuth, titanium and the like, which may contain additions of metalloorganic compounds of precious metals dissolved in organic solvents. The color of the liquid luster preparation usually bears no semblance to the desired optical filter hue resultant from subsequent heat transformation. While luster preparations are available commercially, their formulary compositions are usually considered to be proprietary with the manufacturer of the product. A metallic luster material suitable for use as the first luster component in this screen structure may be, for example, a greenproducing luster material, such as A-1128, which is commercially available from Hanovia Liquid Gold Division, Englehard Industries, Incorporated, East Newark, N.J. The proportional composition of the primary coating mixture is adapted to provide adequate functioning of the photo-resist in conjunction with the amount of luster material required to provide the desired attenuation of the resultant luster filter component. Appropriate proprietary thinners for the respective photo-resist and luster materials are added as desired to adjust the viscosity of the coating mixture to expedite efficient application thereof over the panel surface. It has been found that a coating viscosity in order of 8 to 10 centipoises is appropriate for spin application of the material when rotating the panel in substantially the range of 90 to 150 rpm, whereupon a uniformly applied coating thickness in the order of 2.5 to 4 microns is achieved.

After drying the coated panel, the aperture pattern mask 15 is positioned in spaced relationship thereto as shown in FIG. 1a. The primary coating is then discretely light exposed by directing actinic radiations "Y" and "Z" from two spaced apart positions 16 and 17 through the multiple apertures in the pattern mask, one of which is shown. The respective directed light beams, originating from sources oriented to expose the second and third window patterns, are sized by the mask aperture 18 whereupon the light impinged second and third window areas, 25' and 27' respectively, of the coating are usually slightly larger than the area of the formative aperture 18. After exposure, the primary coating is developed, whereupon the exposed areas thereof, being

polymerically degraded by the uv radiation, are removed to define open second and third filter window patterns in the primary coating. The development material used in this instance is one such as a proprietary liquid developer designated as AZ303, which is commercially available from the aforesigned Shipley Company. A suitable developer concentration is, for example, one part of developer combined with four parts of water. Upon development, the panel is rinsed with water to remove any residual development materials.

The next step in the process involves heating the panel with the patterned luster film thereon in a controlled oxygen atmosphere at a temperature in the region of 450° to 500° Centigrade. This baking or firing thermally decomposes the resist component of the primary coating mixture and oxidizes the first or green-producing luster material changing the color thereof to transform and adhere a substantially continuous and transparent glassy primary layer 21 of green-hued "g" first optical filter material having open second and third filter windows 25 and 27 respectively, formed therein. Reference is directed to FIGS. 1b and 2. The required thickness of the transformed green-hued luster filter material is extremely thin being less than 0.5 microns. It has been found that the thickness of the respective optical filter materials comprising the layered screen should each exhibit a light transmission in the order of 60 percent to provide the desired opacity of the interstitial webbing.

The discretely patterned panel, having the primary layer 21 of filter material adhered thereon, is next coated with a secondary layer 29 of another liquid mixture including the aforescribed positive photosensitive resist material and a second color-producing organometallic luster compound. The second luster filter material may be, for example, a blue-producing composition such as No. 130-F, which is also available from Englehard Industries. With reference to FIG. 1c, the coated panel is then dried and exposed to specific actinic radiations "X" and "Z" emanating from two spaced-apart positions, not shown, oriented to produce the first and third pattern areas, the light therefrom being directed through the apertures of the mask to impinge and degrade the resist coating in those areas 33' and 37' of the secondary coating 29 subsequently occupied by the first and third arrays of filter windows. The exposed secondary coating is then developed with positive photoresist developer as previously described, whereupon the areas of polymerically-degraded exposed coating material 33' and 37' are removed from the first and third pattern window areas. The secondary coating 29 fills in the second window openings 25 in the primary filter layer 21. In referring to FIGS. 1d and 3, after rinsing and drying, the panel is again subjected to heating in a controlled oxygen atmosphere in the temperature range of 450° to 500° Centigrade to thermally decompose the resist portion of the secondary coating mixture and oxidize the second luster material. This baking procedure transforms and adheres a substantially continuous and transparent glassy secondary layer of the second optical filter material 31 having an open third filter window 37 therein and an open first filter window 33 which defines and displays a first filter element area 24 of the first optical filter material 21 therebeneath. The second window opening 25 in the primary filter layer 21, having the secondary filter material disposed therein, defines the second filter element 26. At

this stage in fabrication, the interstitial region 47 is comprised of two uniform layers of filter materials.

The panel having the two patterned filter layers 21 and 31 disposed thereon in a superposed manner is next coated with a tertiary layer of still another liquid mixture 39 incorporating the previously mentioned positive photoresist material and a third organometallic luster compound. The luster preparation for this third filter layer may, for example, be a red-producing luster such as Red Rose No. 9736 or Ruby Red No. 9761, such compositions being commercially available from Englehard Industries. In referring to FIG. 1e, after drying, the tertiary coating is exposed by directing controlled actinic radiations "X" and "Y" from two positions, i.e., the first and second window exposure orientations, through the patterned mask to effect specific degradation of discrete areas 43' and 45' of the tertiary positive resist coating 39 in the areas already occupied by the underlying first and second patterned filter elements 24 and 26 respectively. Developing the exposed tertiary coating removes the degraded exposed areas 43' and 45' of that coating material which had been disposed over the first and second filter elements 24 and 26. After rinsing and drying, the panel is again heated in a controlled oxygen atmosphere to thermally decompose the resist component of the tertiary coating mixture and oxidize the third luster material 39. This heating transforms and adheres a substantially continuous and transparent glassy tertiary layer of the third or red optical filter material 41 having open first 43 and second 45 filter windows therein for displaying the first and second optical filter elements 24 and 26. The third filter element 36 associated with the tertiary layer 41 is defined by the third patterned superimposed open windows 27 and 37 previously formed in the primary and secondary filter layers. Such is evidenced in FIGS. 1f and 4. The superimposed primary 21, secondary 31, and tertiary 41 filter layers being of primary colors, namely green "g", blue "b" and red "r" filtering components provide in combination a substantially opaque uniform interstitial webbing 49 fully surrounding each of the respective round filter windows in the screen structure 11. Each filter window is evenly defined by a uniform peripheral encompassment that is free of indentations.

With reference to FIGS. 1g and 5, upon completing fabrication of the interstitially defined multi-windowed optical filter screen structure as hereinbefore described, the respective green "G", red "R" and blue "B" cathodoluminescent phosphor elements are suitably disposed as a patterned screen 53 over the appropriate "g," "r," and "b" filter windows. Deposition of the pattern of color-emitting phosphor elements, is accomplished in a conventional manner by one of the procedures well known in the art. Therefore, further details of the phosphor screening process will not be considered herein.

It may be expedient from the standpoint of phosphor brightness and color emission, to form a multi-windowed screen structure wherein only one or two of the window areas have the respective optical filter materials disposed therein. Whether or not a filter material is evidenced in a defined window area of the structure is determined by the selection of the light exposure positions during fabrication; for example, if it is found beneficial to have a window area open or free of discrete optical filtering material, that window area has specific actinic radiation directed to it during each of the primary, secondary and tertiary filter layer exposures.

It may be desired to modify the sizes of the apertures in the patterned mask member either before or after forming of the screen structure; as for example, having filter window openings in the opaque interstitial webbing that are smaller than the associated apertures in the patterned mask member subsequently utilized in the operable tube. In one consideration, the mask apertures initially utilized in forming the filter windows and the defining interstitial webbing, may be subjected to a subsequent chemical etching process to enlarge their sizes thereby effecting the desired dimensional differential between the final sized apertures used in tube operation and the initially sized apertures utilized in forming the windows in the interstitial webbing. Prior art is replete with a variety of techniques for modifying the sizes of the pattern mask apertures utilized in the forming of or the operation of specific types of color screen structures. There are several disclosures wherein changing of the aperture sizes is executed by deposition within the aperture openings of peripheral fillin substances applied, as for example, by painting, dipping, electrophoresis, electroplating and vaporization. Such modifications of the apertures of the mask member, may be utilized as desired in conjunction with the screen structure of the invention.

Thus there is provided an improved color cathode ray tube screen structure that incorporates smoothly defined optical filter elements therein which are surrounded by an opaque interstitial webbing of uniform thickness. Uniformity of the opaque interstitial encompassment provides enhanced absorbency of the ambient light thereby effecting improved contrast of the color display.

While there have been shown and described what are at present considered the preferred embodiments of the invention, it will be obvious to those skilled in the art that various changes and modifications may be made therein without departing from the scope of the invention as defined by the appended claims.

What is claimed is:

1. An improvement in a discretely patterned multi-window color screen structure disposed on the inner surface of a cathode ray tube viewing panel, whereof each of the window areas exhibits a peripherally defined smoothness free of indentations such being similar to the shape of the apertures of a related pattern mask member, said improvement comprising:
  - a substantially continuous and substantially transparent primary layer of a first heat formable optical filter material of a first specific hue adhered to the inner surface of said panel, said primary layer having second and third patterns of related window areas formed therein each being free of peripheral indentations;
  - a substantially continuous and substantially transparent secondary layer of a second heat formable optical filter material of a second specific hue, superposed on said primary layer and the second of said window pattern areas formed therein, to provide a single-layer array of window defined second filter elements of said second specific hue in said screen structure, said secondary layer having first and third patterns of discrete window areas formed therein whereof the first window pattern array defines areal portions of said primary layer to provide a single-layer array of first filter elements of said first specific hue in said screen structure that are free of peripheral indentations, said third win-

dow pattern in said secondary layer being superposed over said third window patterns in said primary layer;

a substantially continuous and substantially transparent tertiary layer of a third heat formable optical filter material of a third specific hue superposed over said secondary layer and said third superposed window pattern areas to provide a single-layer array of third filter elements of said third specific hue in said screen structure, said tertiary layer having open first and second window patterns superposed on like respective window areas in said primary and secondary layers, said superimposed primary, secondary and tertiary layers being combined uniformly to provide a substantially opaque uniform interstitial webbing fully surrounding each of the respective filter windows in the screen structure by uniform peripheral encompassment free of indentations; and

three patterns of related cathodoluminescent phosphor elements of first, second and third hues substantially similar to the hues of said first, second and third single-layer filter elements, each pattern of phosphor elements being disposed on a respective single-layer pattern of evenly defined optical filter window elements of substantially like hue.

2. In an improved patterned multi-element color screen structure according to claim 1 wherein each of said optical filter windows is defined as a substantially circular area having a substantially smooth periphery.

3. In an improved pattern multi-element color screen structure according to claim 1 wherein each array of said optical filter elements is formed of at least one appropriate organometallic luster material.

4. An improved patterned multi-element color screen structure according to claim 1 wherein the separate arrays of optical filter elements respectively exhibit a relatively high efficiency for the transmission of radiant energy in selected color regions of the visible spectrum to augment purity of the color output of the respective cathodoluminescent phosphor materials associated with the separate filter arrays.

5. In a color picture tube having a plurality of sets of interleaved spaced phosphor elements disposed on a glass panel, the elements of each set being excitable by an electron beam to emit light of a particular one of a

plurality of primary colors, the improvement comprising a plurality of color transmissive filters each exhibiting light transmission characteristics corresponding to one of the primary colors of said phosphor elements, a single color filter of a corresponding color being disposed between each phosphor element and said glass panel, and an outer-light absorber disposed on the glass panel and filling in the entire interspace between the phosphor elements, said outer-light absorber being formed entirely as a stack of color filters corresponding to each of the primary colors of said phosphor elements.

6. The combination defined in claim 5 wherein each of the color filters is formed as a layer in the glass panel containing colloidal metal reduced and grown from metal ions corresponding to the color of the filter.

7. A colour picture tube comprising a number of phosphor elements of three kinds emitting light of the three primary colours, red, green and blue, respectively, formed on the inner face of the panel glass of the colour picture tube, three kinds of colour filters corresponding to the colours of the light emitted by the phosphor elements arranged at the positions of the phosphor elements, respectively, between the phosphor elements and the panel glass, and an outer-light absorber filled in the interspace between the phosphor elements, in which a first kind of colour filter of the three kinds of colour filters is part of a first colour glass layer corresponding to a first colour of the three primary colours formed on the entire face of the panel glass except for the positions at which phosphor elements emitting light of second and third colours are formed, a second kind of colour filter of the three kinds of colour filters is part of a second colour glass layer corresponding to the second colour of the three primary colours formed on the entire face of the panel glass except for the positions at which phosphor elements emitting light of the first and third colours are formed, a third kind of colour filter of the three kinds of colour filters is a part of a third colour glass layer corresponding to the third colour of the three primary colours formed on the entire face of the panel glass except for the positions at which phosphor elements emitting light of the first and second colours are formed, and the outer-light absorber is the stack of the first, second and third colour glass layers.

\* \* \* \* \*